

## UNITED STATES PATENT OFFICE

1,975,113

## HEAT TREATMENT OF COPPER-BERYLLIUM ALLOYS

Georg Masing, Berlin, and Otto Dahl, Berlin-Charlottenburg, Germany

No Drawing. Application October 22, 1931,  
Serial No. 570,504. In Germany May 21,  
1926

17 Claims. (Cl. 148—21.2)

This invention relates to improvements in heat treatment of copper-beryllium alloys; and it comprises a method of producing certain desired properties, hardness, strength, etc., in copper-beryllium alloys having a major proportion of copper with a beryllium content ranging up to 12 per cent, such alloys at times containing small amounts of other constituents such as phosphorus, tin, zinc, iron, cobalt, aluminum, etc.; said method comprising heating such a copper-beryllium alloy to temperatures somewhat above a transition point lying at about 580° to 600° C., quenching and thereafter heating at temperatures below the said transition point, say at temperatures from 150° to 500° C. for a time; said heating operations being sometimes used individually and sometimes in the succession given, the choice depending on the specific alloy treated and the particular results desired; all as more fully hereinafter set forth and as claimed.

In a prior and copending application, Serial No. 191,263, filed May 13, 1927, of which the present application is a continuation in part, we have described methods for heat treating copper-beryllium alloys and the properties of various alloys of this type; the alloys being specifically described and claimed. In a prior patent No. 1,685,570, we have described and claimed processes for heat treating beryllium-nickel alloys in which nickel predominates. The present application is directed to copper-beryllium alloys of the type in which copper predominates and relates particularly to methods for heat treating such alloys.

While various alloys of beryllium have been mentioned in the art, but little has been published concerning their properties. And it has been found that certain of these alloys have properties which make them particularly adapted for certain technical uses. Beryllium is one of the lightest metals employed technically and it is a good hardening agent in alloys. The hardness imparted to an alloy by the introduction of small proportions of beryllium is characteristic. Copper hardened by alloying with beryllium is a particularly useful material for technical purposes. By methods hereinafter described certain properties of copper-beryllium alloys may be varied at will. For example the hardness may be increased to that of hardened steel or reduced to a point at which the alloy may be readily worked.

The copper-beryllium alloys with which the present invention is most particularly concerned have a beryllium content ranging from about 0.3 up to 12 per cent; the residue being copper or

mainly copper. These alloys can be roughly divided into two ranges, according to their characteristics, (1) alloys from which a so-called "beta modification" separates from a melt and (2) alloys where the "beta modification" does not separate from a melt. It may be said that the beta modification separates upon solidification of alloys having, roughly, a beryllium content of from 5 to 12 per cent, while alloys having a lower content do not show such separation. The lower limit of the existence of the beta modification, however, is altered by the presence of other alloying materials. Thus, in some instances, the beta modification has been found to exist at compositions representing a beryllium content of as low as 3 per cent, when other materials were present.

We have found that these copper-beryllium alloys may be hardened in a two-step process comprising heating at an elevated temperature for some time, followed by quenching and thereafter by "age-hardening" or tempering at a lower temperature for a time sufficient to improve their properties. But each step of this process can also be employed alone to produce advantageous results under some circumstances.

Alloys having a beryllium content below that permitting existence of the beta modification, that is, roughly, below 3 to 5 per cent, are advantageously hardened by heat treating at temperatures above a certain transition point, which appears to lie at approximately 580° to 600° C. followed by "age-hardening" below this temperature. Thus, the alloy may be first heated at any convenient temperature between the transition point and the melting point, that is advantageously somewhat above 600° C., followed by cooling. Small pieces cool with sufficient rapidity in the air while large pieces should be quenched. This process is followed by a prolonged heating at temperatures below the transition point, such as from 150° to 500° C. This heating is continued for a time sufficient to improve the properties of the alloys. At the lower temperatures several days may be required for this treatment, while at 300° C. two hours is sufficient. In a specific example of such a heat treatment, an alloy of 97 per cent copper and 3 per cent beryllium, having an initial hardness of about 125° Brinell, was found to have a final hardness of about 360° Brinell.

Throughout the range of the existence of the beta modification the heat treatment required to produce the maximum hardness comprises merely the first step of the above described process, namely a heating to temperatures above the

60

65

70

75

80

85

90

95

100

105

110

transition point followed by quenching. The second step, namely heating below the transition point may be advantageously employed to obtain the alloy in a relatively soft and mechanically workable condition. In one case a copper-beryllium alloy containing 6.7 per cent of beryllium was found to have a hardness of 490 in the chilled casting. This hardness was increased to 730 by heat treatment above 580° C., followed 10 by quenching.

Upon a subsequent prolonged heat treatment at temperatures below 580° C. the hardness of the above mentioned alloy was reduced to about 240° Brinell. This latter treatment increases the ductility and toughness of the alloy. However, it 15 may be worked readily while in this condition.

The above described heat treatments can be applied to both cast and to mechanically worked alloys. In the case of cast alloys the heat treatment at the higher temperatures may usually be obviated, the cooling in the casting taking the place of this treatment. A chilled casting may be merely reheated between 150° and 300° C.

For the production of alloys having intermediate properties between the extremely hard and the workable types there are two methods available. The first method consists in a heat treatment at intermediate temperatures, for example between 450° and 600° C. The second method 20 consists of a prolonged heat treatment at somewhat lower temperatures. This latter procedure is somewhat similar to the final step of the usual two-step process. A preliminary mechanical working operation is frequently advantageous before the heating step.

The first effect of a prolonged heating at temperatures below the transition point is to harden the alloy, but this is followed by the production of high ductility and toughness as well as a high tensile strength. Since the heating may be interrupted at any point, it is possible in this way to produce alloys having, within wide limits, almost any desired properties. Definite values of hardness, ductility, toughness and strength may be 40 produced. Somewhat similar results to the above may be obtained by heating the alloy above 600° C. followed by a slow cooling. This method is not as conveniently controlled, however.

In one particular example of the above heat 50 treatment a copper-beryllium alloy, with a beryllium content of 2.5 per cent was heated at 500° C. for some time. The alloy was then found to possess a notched bar toughness of about 15 meter-kilograms per square centimeter and a tensile strength of 75 kilograms per square millimeter. This same alloy, after being treated by the two-step process, namely by heating above 600° C. and then at temperatures in the neighborhood of 450° C., gave a notched bar test toughness of only 1 55 meter-kilogram per square centimeter and was found to have a tensile strength of 140 kilograms per square millimeter. It has been found that advantageous results with the above described single heating at the lower temperatures are only 60 obtained when the beryllium content of the alloy amounts to at least 1 per cent.

The effect of added bodies upon the properties of the alloys and upon the heat treatments required is very striking. The addition of up to 1 70 per cent of phosphorus has been found to produce a considerable reduction in the amount of beryllium metal required to produce certain improved characteristics. The time required for heat treatment is reduced by the presence of 75 phosphorus. Other metals such as zinc, tin,

aluminum and magnesium may be present simultaneously in the alloy with the production of improved properties.

A typical heat hardening process, as carried out with an alloy containing 0.25 per cent of phosphorus and about 1.5 per cent of beryllium, may be carried out as follows: The alloy is heated above the previously mentioned transition point, say at 800° C., and then quickly cooled. After cooling the hardness of one particular sample was found to be only 80° Brinell. By subsequently tempering the alloy by heating for an hour at 350° C., the hardness was increased to 210° Brinell.

In comparison with the above, when a copper-beryllium alloy of the same beryllium content but free from phosphorus was treated in the same manner, the hardness, on cooling from 800° C., was found to be 74° Brinell and, upon heating for as long as 7 hours at 350° C., the hardness increased only 20° Brinell. The beneficial effects of the phosphorus addition is evident.

The beryllium content can be reduced without detriment when addition metals, such as aluminum, tin, silver and magnesium, are present in the alloy. Alloys of this type contain up to about 2.5 per cent of beryllium, a somewhat larger per cent of one of these other metals and a preponderating amount of copper; 5 to 10 per cent of addition metals, for example, produces desirable 105 results.

We have found that the addition of metals other than copper and beryllium permits the reduction of the beryllium content to a fraction of the amount required when only copper and 110 beryllium are employed; these other metals act, so to speak, to reinforce or assist the action of beryllium. Since beryllium is by far the most expensive of the metallic constituents, a reduction in the quantity required is advantageous. For example, when copper only is alloyed with the beryllium at least 1 per cent of beryllium must be present in order to give an alloy with a high degree of hardness. But, upon the addition of from 5 to 25 per cent of one of the other metals 120 mentioned, the beryllium content may be reduced to about 0.3 per cent to obtain the same degree of hardness.

The heat treatment required for these multi-metal alloys is similar to that described previously. The two-step process is advantageous.

The properties of the above described copper-beryllium alloys, including within this term alloys which may contain one or more additional metals, fit them for many special technical uses. The 130 alloys are especially suited for making metallic springs, whether of leaf, helical or spiral form. The use of such springs in instruments of precision is highly advantageous due to their high resistance to corrosion and permanent characteristics. The use of the described alloys in electrical instruments is desirable, especially where there is frictional contact, for example in knife switches, commutators, slip rings, bearings, sliding contact points, etc.

By the terms "remainder substantially copper" and "balance substantially copper", occurring in the claims, we mean that the alloys called for may also contain small amounts of addition metals acting to reinforce the hardening effect of 145 the beryllium, these metals, including phosphorus, tin, zinc, iron, cobalt and aluminum occurring in amounts insufficient to substantially alter the characteristic properties of the said alloys.

What we claim is:

1. In the heat treatment of copper-beryllium alloys containing from about 0.3 to 12 per cent by weight of beryllium with the remainder substantially copper, the process which comprises heating such an alloy at temperatures above a transition point, which lies in the neighborhood of 580° to 600° C., but below its melting point, quenching and age-hardening by prolonged heating at temperatures above about 150° C. but below said transition point. 50
2. In the heat treatment of copper-beryllium alloys containing from about 0.3 to 12 per cent by weight of beryllium with the remainder substantially copper, the steps which comprise heating such an alloy at temperatures below its melting point but above about 580° C. and subsequently quenching. 55
3. In the heat treatment of copper-beryllium alloys containing from about 0.3 to 12 per cent by weight of beryllium with the remainder substantially copper, the step which comprises tempering such an alloy by a prolonged heating at temperatures below about 580° to 600° C. but above about 150° C. 60
4. The process of heat treating copper-beryllium alloys having a beryllium content above about 0.3 per cent but below percentages at which the beta-modification separates upon solidification, ranging from about 3 to 5 per cent by weight, with a balance substantially copper, which comprises heating such an alloy at temperatures below its melting point but above about 600° C., and age-hardening by heating at temperatures ranging from about 150° to 500° C. until its physical properties have been improved. 65
5. In the heat treatment of copper-beryllium alloys containing sufficient beryllium to cause separation of the beta-modification upon solidification, ranging from about 3 per cent to 12 per cent by weight, with a balance substantially copper, the process which comprises heating such an alloy at temperatures below its melting point but above about 600° C. and quenching. 70
6. The process of claim 5 in which the alloy is further heated at temperatures between 150° to 500° C. in order to produce workable properties. 75
7. In the heat treatment of copper-beryllium alloys containing from 0.3 to 12 per cent by weight of beryllium, with a balance substantially copper, the process which comprises heating such an alloy for a prolonged interval at temperatures between about 450°-600° C. to produce high ductility and toughness. 80
8. The process of claim 7 wherein the heating step is preceded with a mechanical working operation. 85
9. The process of claim 3 in which the temperature of the tempering step lies between 150° and 500° C. 90
10. In the heat treatment of copper-beryllium alloys containing from about 0.3 to 12 per cent by weight of beryllium with a balance substantially copper, the process which comprises chill-casting such an alloy and reheating to temperatures between 150° and 500° C. until the physical properties have been improved. 95
11. The process of claim 1 wherein the copper-beryllium alloy also contains from about 0.1 to 1 per cent of phosphorus. 100
12. The process of claim 2 wherein the copper-beryllium alloy also contains from about 0.1 to 1 per cent of phosphorus. 105
13. The process of claim 3 wherein the copper-beryllium alloy also contains from about 0.1 to 1 per cent of phosphorus. 110
14. The process of claim 4 wherein the copper-beryllium alloy also contains from about 0.1 to 1 per cent of phosphorus. 115
15. The process of claim 5 wherein the copper-beryllium alloy also contains from about 0.1 to 1 per cent of phosphorus. 120
16. The process of claim 7 wherein the copper-beryllium alloy also contains from about 0.1 to 1 per cent of phosphorus. 125
17. The process of claim 10 wherein the copper-beryllium alloy also contains from about 0.1 to 1 per cent of phosphorus. 130

GEORG MASING. 120  
OTTO DAHL. 125

50

125

55

130

60

135

65

140

70

145

75

150